# EUROPEAN PATENT SPECIFICATION

(11) **EP 4 354 475 B1**
(45) Date of publication and mention of the grant of the patent: **22.04.2026**
(21) Application number: 23202376.2
(22) Date of filing: 09.10.2023
(51) Int. Cl.: H01F 41/02, H01F 1/057

(54) **METHOD FOR IMPROVING THE COERCIVITY OF A NEODYMIUM-IRON-BORON MAGNET AND MAGNET OBTAINED BY THE METHOD**
VERFAHREN ZUR VERBESSERUNG DER KOERZITIVKRAFT EINES NEODYM-EISEN-BOR-MAGNETEN UND DURCH DAS VERFAHREN ERHALTENER MAGNET
PROCÉDÉ D'AMÉLIORATION DE LA COERCITIVITÉ D'UN AIMANT NÉODYME-FER-BORE ET AIMANT OBTENU PAR LE PROCÉDÉ

(30) Priority: 10.10.2022 CN 202211239979
(43) Date of publication of application: 17.04.2024
(73) Proprietor: Yantai Dongxing Magnetic Materials Inc., Yantai City 265500 (CN)
(72) Inventor: Yang, Kunkun, Yantai City, 265500 (CN); Peng, Zhongjie, Yantai City, 265500 (CN); Wang, Chuanshen, Yantai City, 265500 (CN); Ding, Kaihong, Yantai City, 265500 (CN)
(74) Representative: Gulde & Partner

(56) References cited:
- US-A1- 2012 139 388
- US-A1- 2013 087 248
- US-A1- 2013 171 342
- US-A1- 2018 166 192

## Description

### Technical Field

The present disclosure relates to the field of production of neodymium-iron-boron magnets, in particular to a method for improving the coercivity of a neodymium-iron-boron magnet and a magnet prepared by the method.

### Background

Sintered neodymium-iron-boron permanent magnets have been widely used in air conditioners, automobiles, medical treatment, industry and other fields. With the development of time, on the one hand, the sintered neodymium-iron-boron permanent magnets are required to have higher miniaturization and lamination level, and on the other hand, the sintered neodymium-iron-boron permanent magnets are required to have higher remanence and coercivity.

The coercivity of the sintered neodymium-iron-boron permanent magnets can be improved by adding terbium and dysprosium to the alloys of the sintered neodymium-iron-boron permanent magnets. However, if terbium and dysprosium are added to the main phase grains by a traditional composition mixing method, the remanence of the permanent magnets is significantly reduced and the method consumes large amounts of heavy rare earth elements.

CN107578912A discloses a process for producing a neodymium-iron-boron magnet having a high coercivity. The method comprises mixing a heavy rare earth powder with an antioxidant, an adhesive and an organic solvent to obtain a suspension, coating a surface of a neodymium-iron-boron magnet with the suspension, and drying the suspension, followed by high temperature diffusion and aging treatment to improve the coercivity of the magnet. The process has a high production efficiency and a high material utilisation rate, so it has been widely used. However, due to low hardness and strength, a heavy rare-earth film produced by this method is easily scratched, resulting in local loss of heavy rare-earth elements, thus impairing the diffusion effect. In addition, such a film coating is prone to irregular shrinkage in diffusion and heating processes, resulting in local loss of the heavy rare earth elements on the surface of the neodymium-iron-boron magnet and excessive accumulation of the heavy rare earth elements in some areas, so that the neodymium-iron-boron magnet has poor property uniformity after diffusion. For example, US 2012/0139388 A1 discloses a rare earth sintered magnet obtained by adhering a rare earth compound to a rare earth sintered magnet body and subjecting the resultant magnet body to heat treatment. US 2018/0166192 A1 relates to a method of producing a rare earth permanent magnet including preparing a NdFeB sintered magnet, coating a surface of the NdFeB sintered magnet with a grain boundary diffusion material including R hydrate or R fluoride, and RₐM_{b}, or M, to form a grain boundary diffusion coating layer, and diffusing the grain boundary diffusion material into a grain boundary of the NdFeB sintered magnet by heat treatment, wherein M is a metal having a melting point higher than a heat treatment temperature during the diffusion, R is a rare earth element.

During the high-temperature diffusion of the coating on the surface of the neodymium-iron-boron magnet, the heavy rare earth elements are oversupplied for a short time, so that excessive amounts of the heavy rare earth elements are consumed by excessive reactions of the surface of the neodymium-iron-boron magnet with the heavy rare earth elements. Meanwhile, due to the insufficient supply, the heavy rare earth elements in the neodymium-iron-boron magnet are poorly dispersed, so that the surface and the centre of the magnet eventually have large differences in properties after diffusion, and excessive amounts of the rare earth elements are consumed.

### Summary of Invention

The invention is defined by the appended claims. The description that follows is subjected to this limitation. Any disclosure lying outside the scope of said claims is only intended for illustrative as well as comparative purposes.

In order to solve the problems that heavy rare earth coatings have low hardness and strength, are easily scratched and worn in a production process, and are prone to shrinkage in a diffusion process, and that heavy rare earth elements have poor diffusion uniformity and high consumption due to excessive supply of the heavy rare earth elements in a short time in the prior art, the present disclosure provides a method for improving the coercivity of a neodymium-iron-boron magnet and a magnet produced by the method.

In order to achieve the above purposes, a method for improving the coercivity of a neodymium-iron-boron magnet includes the following steps:
(S1) subjecting a heavy rare earth diffusion source powder, an organic adhesive, a spherical high-temperature resistant ceramic powder and an organic solvent to mixing and stirring to prepare a heavy rare earth slurry, wherein the particle size of the spherical high-temperature resistant ceramic powder is required to be 5 to 10 times of that of the diffusion source powder, and the weight of the spherical high-temperature resistant ceramic powder is 10% to 30% of that of the heavy rare earth diffusion source powder;
(S2) coating a surface of a neodymium-iron-boron magnet with the heavy rare earth slurry and drying the heavy rare earth slurry to form a heavy rare earth coating; and
(S3) subjecting the neodymium-iron-boron magnet coated with the heavy rare earth coating to high-temperature diffusion and aging treatment under vacuum or argon protection conditions.

The heavy rare earth coating formed in step (2) may have a basic (skeletal) structure composed of the spherical high-temperature resistant ceramic powder, and the heavy rare earth diffusion source powder is distributed in the interstices of the three-dimensional network provided by the basic structure. In other words, the heavy rare earth diffusion source is located in free spaces that arise between the larger spherical high-temperature resistant ceramic particles.

Preferably, in step (S1), the heavy rare earth diffusion source powder is at least one of a pure terbium powder, a pure dysprosium powder, a dysprosium hydride powder and a terbium hydride powder, and the heavy rare earth diffusion source powder has an average particle size in a range of 2 to 10 µm.

The average particle diameter (D50) of the particles may be measured by laser diffraction (LD). The method may be performed according to ISO 13320:2020. According to the IUPAC definition, the equivalent diameter of a non-spherical particle is equal to a diameter of a spherical particle that exhibits identical properties to that of the investigated non-spherical particle.

Preferably, in step (S1), the organic adhesive is a resin adhesive or a rubber adhesive.

The organic solvent may be acetone, s-butyl acetate, ethylbenzene or a combination thereof.

Preferably, in step (S1), the spherical high-temperature resistant ceramic powder is at least one of a spherical alumina ceramic powder, a spherical zirconia ceramic powder and a spherical boron nitride ceramic powder; and the spherical high-temperature resistant ceramic powder has an average particle size in a range of 10 to 100 µm.

Preferably, in step (S1), the total weight of the heavy rare earth diffusion source powder and the spherical high-temperature resistant ceramic powder is 40% to 80% of the weight of the heavy rare earth slurry, the weight of the organic adhesive is 5% to 10% of the weight of the heavy rare earth slurry, and the organic solvent is the residual.

Preferably, in step (S2), the heavy rare earth slurry is coated by screen printing or spraying.

Preferably, in step (S2), the weight of the heavy rare earth diffusion source powder in the heavy rare earth coating coated on the surface of the neodymium-iron-boron magnet is 0.3% to 1.5% of the weight of the neodymium-iron-boron magnet.

Preferably, in step (S3), the high-temperature diffusion is performed at a temperature of 850 to 950°C for 3 to 48 h; and the aging treatment is performed at a temperature of 450 to 650°C for 3 to 10 h.

A magnet having a high coercivity can be obtained by the method. The heavy rare earth coating includes a basic structure composed of the spherical high-temperature resistant ceramic powder and a heavy rare earth diffusion source powder filled in the interstices of the basic structure.

The method for improving the coercivity of a neodymium-iron-boron magnet and the magnet obtained by the method cause at least the following technical effects.
(1) A certain proportion of the spherical high-temperature resistant ceramic powder having a defined particle size is added to the heavy rare earth slurry and then coated and dried to form a heavy rare earth coating with a special structure. The special structure includes a basic (skeletal) structure composed of the spherical high-temperature resistant ceramic powder. The heavy rare earth diffusion source particles are distributed in a continuous three-dimensional network shape in gaps of the basic structure. By means of said basic structure, on the one hand, the overall hardness and strength of the coating layer are improved, and the wear resistance and scratch resistance of the coating layer are enhanced. On the other hand, shrinkage of the heavy rare earth coating layer during the diffusion and heating processes is prevented, so that heavy rare earth elements are distributed more uniformly in the diffusion process.
(2) The heavy rare earth diffusion source in the heavy rare earth coating is distributed homogeneously in gaps of the basic structure given by the spherical high temperature resistant ceramic powder. Therefore, the heavy rare earth diffusion source diffuses continuously and stably into the neodymium-iron-boron magnet along the gaps of basic structure during the high-temperature diffusion process. Thereby, an excessive supply of the heavy rare earth diffusion source in a short term is avoided, the diffusion property and the diffusion uniformity are improved, and waste of the heavy rare earth elements is reduced. In addition, the heavy rare earth components in the heavy rare earth coating layer are divided by the spherical ceramic powder to form a uniform and continuous network-shaped distribution, so that the diffusion of oxygen from an outer surface of the coating to the inside of the coating in an atmospheric environment is slowed down, and the oxidation resistance of the heavy rare earth coating is improved.
(3) In the coating process, due to the addition of the spherical ceramic powder, the fluidity and suspensibility of the slurry are improved, and thereby the coating precision and the coating stability are improved. In addition, due to the increase of the ceramic powder, degassing channels in the heavy rare earth elements are improved, which are suitable during volatilization of the organic solvent and the like during the drying of the coated heavy rare earth slurry. Thereby, the production stability is improved.

### Brief Description of the Drawings

FIG. 1 is a schematic diagram of a neodymium-iron-boron magnet coated with a heavy rare earth coating on a surface.
FIG. 2 is a schematic diagram of a neodymium-iron-boron magnet cut in a diffusion direction.

### Detailed Description of the Embodiments

Reference will now be made in detail to embodiments, examples of which are illustrated in the accompanying drawings. Effects and features of the exemplary embodiments, and implementation methods thereof will be described with reference to the accompanying drawings. In the drawings, like reference numerals denote like elements, and redundant descriptions are omitted. The present disclosure, however, may be embodied in various different forms, and should not be construed as being limited to only the illustrated embodiments herein. Rather, these embodiments are provided as examples so that this disclosure will be thorough and complete, and will fully convey the aspects and features of the present disclosure to those skilled in the art.

FIG. 1 is a schematic diagram of a neodymium-iron-boron magnet 1 coated with a heavy rare earth coating on its outer surface. The heavy rare earth coating includes a spherical high-temperature resistant ceramic powder 2 and a heavy rare earth diffusion source 3 embedded in the basic structure provided by the particles of the spherical high-temperature resistant ceramic powder 2.

### Example 1

(S1) A total of 4 raw components, including a pure Tb powder with an average particle size D50 of 2 µm as a heavy rare earth diffusion source, an isoamyl rubber adhesive, acetone as solvent and a spherical alumina ceramic powder with an average particle size D50 of 10 µm were used as raw materials of the heavy rare earth slurry. First, the pure Tb powder was mixed with the spherical alumina ceramic powder, wherein the weight of the spherical alumina ceramic powder was 10% of the weight of the pure Tb powder. The obtained powder mixture, the rubber adhesive and acetone were mixed in weight proportions of 40%, 5% and 55%, respectively, and stirred evenly to prepare the heavy rare earth slurry.

(S2) The heavy rare earth slurry was coated on two surfaces (10*10 mm) of a neodymium-iron-boron magnet with a size of 10*10*5 mm by screen printing and dried to form a heavy rare earth coating, wherein the weight ratio of heavy rare earth elements in the coating to the neodymium-iron-boron magnet was controlled to 0.8%. The neodymium-iron-boron matrix of the magnet was obtained by performing processes such as melting, pulverizing, molding, sintering and aging to obtain an N48H NdFeB magnet and then performing machining and had a size of 10*10*5 mm. Grade N42H refers to a specific type of neodymium magnet strength rating. The "N" in the grade stands for neodymium, while the number following it refers to the strongest point of the material's B-H curve or its maximum energy product (in MGOe). For grade N42H, the maximum energy product of the magnet is 42 MGOe, which makes it a high-performance magnet with strong magnetic force. The "H" in the grade refers to the magnet's high resistance to temperature, which can operate up to 120 degrees Celsius.

(S3) The neodymium-iron-boron magnet coated with the heavy rare earth coating was subjected to diffusion and aging under vacuum conditions, wherein the diffusion and aging processes were performed at a temperature of 850°C for 48 h and at a temperature of 500°C for 5 h, respectively. Then, overall magnetic properties of a product obtained after the diffusion was completed were tested.

The product obtained after the diffusion was evenly cut into 5 pieces in a diffusion direction, and magnetic properties of magnets at different positions in the diffusion direction after the diffusion were tested.

### Comparative Example 1

(S1) A total of 3 raw components, including a pure Tb powder with an average particle size of 2 µm as a heavy rare earth diffusion source, an isoamyl rubber adhesive and acetone as solvent were used as raw materials of a heavy rare earth slurry. The pure Tb powder diffusion source, the rubber adhesive and the solvent were mixed in weight proportions of 40%, 5% and 55%, respectively, and stirred evenly to prepare the heavy rare earth slurry.

(S2) The heavy rare earth slurry was coated on two surfaces (10*10 mm) of a neodymium-iron-boron magnet with a size of 10*10*5 mm by screen printing and dried to form a heavy rare earth coating, wherein the weight ratio of heavy rare earth elements in the coating to the neodymium-iron-boron matrix was controlled to 0.8%. The neodymium-iron-boron matrix was obtained by performing processes such as melting, pulverizing, molding, sintering and aging to obtain an N48H brand blank and then performing machining and had a size of 10*10*5 mm.

(S3) The neodymium-iron-boron magnet coated with the heavy rare earth coating was subjected to diffusion and aging under vacuum conditions, wherein the diffusion and aging processes were performed at a temperature of 850°C for 48 h and at a temperature of 500°C for 5 h, respectively. Then, overall magnetic properties of a product obtained after the diffusion was completed were tested.

The product obtained after the diffusion was evenly cut into 5 pieces in a diffusion direction, and magnetic properties of magnets at different positions in the diffusion direction after the diffusion were tested.

In order to compare the scratch resistance of the heavy rare earth coatings in Examples and Comparative Examples, a mutual friction experiment was carried out. The proportions of the exposed areas of the matrices in the total coating areas were statistically calculated after scratching the heavy rare earth coating layers on the surfaces of the samples prepared by Example 1 and Comparative Example 1, and the statistical data were recorded in Table 1 and designated as the scratch ratio.

In order to compare the shrinkage resistance of heavy rare earth coatings in examples and comparison examples in a high-temperature diffusion process, 100 pieces of diffusion samples in Example 1 and Comparison Example 1 were taken separately, proportions of samples having a shrinkage phenomenon of heavy rare earth film layers after diffusion in total statistical numbers were calculated by statistics, and statistical data were recorded in Table 1 and named as shrinkage ratio.

Furthermore, magnetic properties of the neodymium-iron-boron magnets prior to the diffusion process and after the diffusion process according to Example 1 and Comparative Example 1 are summarizes in Table 1.

**Table 1 Comparison of properties of magnets obtained in Example 1 and Comparative Example 1**

| Sample | Scratch ratio | Shrinkage ratio | Br (T, kGs) | Hcj (kA/m, kOe) | Hk/Hcj |
|---|---|---|---|---|---|
| uncoated magnet | / | / | 13.8, 13.8 | 1361.16, 17.10 | 0.982 |
| Example 1 | 0% | 0% | 13.62, 13.62 | 2189, 27.50 | 0.975 |
| Comparative Example 1 | 20% | 7% | 13.60, 13.60 | 2141.24, 26.90 | 0.968 |

From Table 1, it can be seen that the sample coated with the heavy rare earth coating of Example 1 is not scratched in the mutual friction experiment. Contrary, the sample of Comparative Example 1 is scratched in a proportion of 20%, indicating that the heavy rare earth coating of Example 1 has a higher scratch resistance. In addition, the heavy rare earth coating on the surface of the sample in Comparative Example 1 shrinks in a proportion of 7% during the high-temperature diffusion process, while the heavy rare earth coating of Example 1 avoids any shrinkage phenomenon when performing the high-temperature diffusion process. Hence, the shrinkage resistance of Example 1 is improved.

From Table 1, it can be further seen that the Br in the magnet after the diffusion in Example 1 is reduced by only 0.018 T [0.18 kGs], the intrinsic coercivity (Hcj) is improved by 827.84 kA/m [10.4 kOe], and the squareness is reduced by 0.007. However, Br in the magnet after the diffusion in Comparative Example 1 is reduced by 0.02 T [0.2 kGs], the Hcj is only improved by 780.08 kA/m [9.8 kOe], and the squareness is reduced by 0.014. Through the above results, it can be seen that properties of the neodymium-iron-boron magnets can be improved by use of the special coating slurry, respectively the obtained coating layer, of Example 1. Example 1 has the advantages that the remanence is less reduced, the coercivity is improved to a higher level, and the squareness is less reduced.

The neodymium-iron-boron magnet before diffusion, the neodymium-iron-boron magnet obtained after the diffusion process in Example 1 and the neodymium-iron-boron magnet obtained after the diffusion was completed in Comparative Example 1 were evenly cut into 5 pieces in the diffusion direction, respectively, and then magnetic properties of these magnets were tested. The magnets after the diffusion were compared in uniformity of properties, as shown in Table 2 below. FIG. 2 is a schematic diagram of the neodymium-iron-boron magnet cut in a diffusion direction. In FIG. 2, 1# and 5# refer to samples on outermost layers in the diffusion direction, and 3# refers to a sample at a central position in the diffusion direction.

**Table 2 Comparison of uniformity of properties of magnets obtained in Example 1 and Comparative Example 1**

| Sample no. | Matrix before diffusion | Example 1 | Comparative Example 1 |
|---|---|---|---|
| | Hcj (kA/m, [kOe]) | Hcj (kA/m, [kOe]) | Hcj (kA/m, [kOe]) |
| 1# | 1361.16, [17.10] | 2228.8, [28.00] | 2228.8, 28.00 |
| 2# | 1361.96, [17.11] | 2109.4, [26.50] | 2085,52, 26.20 |
| 3# | 1361.16, [17.10] | 2053.68, [25.80] | 1997,96, 25.10 |
| 4# | 1362.75, [17.12] | 2117.36, [26.60] | 2078,36, 26.11 |
| 5# | 1361.96, [17.11] | 2220.84, [27.90] | 2212,88, 27.80 |

From Table 2, it can be seen that under same weight gain conditions of heavy rare earth elements and diffusion process conditions, the difference of the coercivity between a sample at an outermost layer position and a sample at a central position of the magnet obtained after diffusion in the diffusion direction in Example 1 is 147.26 kA/m [1.85 kOe], and the Hcj of the sample at a central position is 692.52 kA/m [8.7 kOe] higher than that of the matrix. The difference of the coercivity between a sample at an outermost layer position and a sample at a central position of the magnet obtained after diffusion in the diffusion direction in Comparative Example 1 is 183.08 kA/m [2.3 kOe], and the Hcj of the sample at a central position is 8 KOe higher than that of the matrix. In addition, the property of the magnet at a central position after diffusion in Example 1 is 55.72 kA/m [0.7 kOe] higher than that of the magnet at a central position after diffusion in Comparative Example 1. Through the above comparison, it can be seen that the magnet in Example 1 has a higher diffusion depth and is diffused more uniformly.

### Example 2

(S1) A total of 4 raw components, including a mixture of a dysprosium hydride powder with an average particle size of 5 µm and a pure dysprosium powder at a ratio of 1:1 as a heavy rare earth diffusion source powder, a polyvinyl chloride resin adhesive, s-butyl acetate as solvent and a spherical zirconia ceramic powder with an average particle size of 35 µm were used as raw materials of a heavy rare earth slurry. First, the heavy rare earth diffusion source powder was mixed with the spherical zirconia powder, wherein the weight of the zirconia ceramic powder was 15% of the weight of the heavy rare earth diffusion source powder. Then, the mixed powder was used as a diffusion source intermediate, and the diffusion source intermediate, the resin adhesive and the ester organic solvent were mixed in proportions of 60%, 10% and 30%, respectively, and stirred evenly to prepare the heavy rare earth slurry.

(S2) The heavy rare earth slurry was coated on two surfaces (10*10 mm) of a neodymium-iron-boron matrix with a size of 10*10*3 mm by screen printing and dried to form a heavy rare earth coating with a special structure, wherein the weight ratio of heavy rare earth elements in the coating to the neodymium-iron-boron matrix was controlled to 0.3%. The neodymium-iron-boron matrix was obtained by performing processes such as melting, pulverizing, molding, sintering and aging to obtain an N55H brand blank and then performing machining and had a size of 10*10*3 mm.

(S3) The neodymium-iron-boron magnet coated with the heavy rare earth coating was subjected to diffusion and aging under the protection of an argon atmosphere, wherein the diffusion and aging processes were performed at a temperature of 900°C for 3 h and at a temperature of 450°C for 3 h, respectively. Then, overall magnetic properties of a product obtained after the diffusion was completed were tested.

The product obtained after the diffusion was completed was evenly cut into 3 pieces in a diffusion direction, and magnetic properties of magnets at different positions in the diffusion direction after the diffusion were tested.

In order to fully illustrate technical advantages of the patent scheme compared with a traditional coating and diffusion scheme, Comparative Example 2 was set below.

### Comparative Example 2

(S1) A total of 3 raw components, including a mixture of a dysprosium hydride powder with an average particle size of 5 µm and a pure dysprosium powder at a ratio of 1:1 as a heavy rare earth diffusion source powder, a polyvinyl chloride resin adhesive and s-butyl acetate as solvent were used as raw materials of a heavy rare earth slurry. The heavy rare earth diffusion source powder, the resin adhesive and the ester organic solvent were mixed in proportions of 60%, 10% and 30%, respectively, and stirred evenly to prepare the heavy rare earth slurry.

(S2) The heavy rare earth slurry was coated on two surfaces (10*10 mm) of a neodymium-iron-boron matrix with a size of 10*10*3 mm by screen printing and dried to form a heavy rare earth coating with a special structure, wherein the weight ratio of heavy rare earth elements in the coating to the neodymium-iron-boron matrix was controlled to 0.3%. The neodymium-iron-boron matrix was obtained by performing processes such as melting, pulverizing, molding, sintering and aging to obtain an N55H brand blank and then performing machining and had a size of 10*10*3 mm.

(S3) The neodymium-iron-boron magnet coated with the heavy rare earth coating was subjected to diffusion and aging under the protection of an argon atmosphere, wherein the diffusion and aging processes were performed at a temperature of 900°C for 3 h and at a temperature of 450°C for 3 h, respectively. Then, overall magnetic properties of a product obtained after the diffusion was completed were tested.

The product obtained after the diffusion was completed was evenly cut into 3 pieces in a diffusion direction, and magnetic properties of magnets at different positions in the diffusion direction after the diffusion were tested.

In order to compare the scratch resistance of heavy rare earth coatings in examples and comparative examples, a mutual friction experiment was carried out by enabling a sample coated with a heavy rare earth coating in Example 2 to get in contact with a coating surface of a sample coated with a heavy rare earth coating with a special structure in Comparative Example 2, proportions of exposed areas of matrices in total coating areas were calculated by statistics after heavy rare earth film layers on the surfaces of the samples in Example 2 and Comparative Example 2 were scratched, and statistical data were recorded in Table 3 and named as a scratch ratio.

In order to compare the shrinkage resistance of heavy rare earth coatings in examples and comparative examples in a high-temperature diffusion process, 100 pieces of diffusion samples in Example 2 and Comparative Example 2 were separately taken, proportions of samples having a shrinkage phenomenon of heavy rare earth film layers after diffusion in total statistical numbers were calculated by statistics, and statistical data were recorded in Table 3 and named as a shrinkage ratio.

Properties of a neodymium-iron-boron magnet before diffusion, overall properties of a neodymium-iron-boron magnet obtained after the diffusion was completed in Example 2 and overall properties of a neodymium-iron-boron magnet obtained after the diffusion was completed in Comparative Example 2 were compared, as shown in Table 3 below.

**Table 3 Comparison of properties of magnets obtained in Example 2 and Comparative Example 2**

| Sample | Scratch ratio | Shrinkage ratio | Br (T, [kGs]) | Hcj (kA/m, [kOe]) | Hk/Hcj |
|---|---|---|---|---|---|
| uncoated magnet | / | / | 1.461, [14.61] | 1235.39, [15.52] | 0.989 |
| Example 2 | 0% | 0% | 1.452, [14.52] | 1538.66, [19.33] | 0.981 |
| Comparative Example 2 | 10% | 11% | 1.451, [14.51] | 1498.07, [18.82] | 0.980 |

From Table 3, it can be seen that the sample coated with a heavy rare earth coating having a special structure in Example 2 is not scratched in the mutual friction test with the sample coated with a heavy rare earth coating in Comparative Example 2, while the sample in Comparative Example 2 is scratched in a proportion of 10%, indicating that the heavy rare earth coating in Example 2 has a higher scratch resistance. In addition, the heavy rare earth coating on the surface of the sample in Comparative Example 2 exhibits a shrinkage phenomenon in a proportion of 11% in a high-temperature diffusion process, while the heavy rare earth coating on the surface of the sample in Example 2 does not exhibit a shrinkage phenomenon in a high-temperature diffusion process, indicating that the heavy rare earth coating with a special structure prepared in Example 2 has a higher shrinkage resistance than the heavy rare earth coating prepared in Comparative Example 2.

From Table 3, it can be seen that under the same heavy rare earth weight gain conditions, the content of Br in the magnet after diffusion in Example 2 is reduced by 0.009 T [0.09 kGs], the Hcj is improved by 303.28 kA/m [3.81 kOe], and the squareness is reduced by 0.008. The Br content in the magnet after diffusion in Comparative Example 2 is reduced by 0.01 T [0.1 kGs], the Hcj is improved by 262,68 kA/m [3.3 kOe] and the squareness is reduced by 0.009. From the above results it can be seen that the properties of the neodymium-iron-boron magnets can be improved by the diffusion schemes in Example 2 and Comparative Example 2. However, under the same heavy rare earth weight gain conditions, the scheme in Example 2 has the advantage of improving the coercivity to a higher level.

The neodymium-iron-boron magnet before diffusion, the neodymium-iron-boron magnet obtained after diffusion in Example 2 and the neodymium-iron-boron magnet obtained after diffusion in Comparative Example 2 were each cut equally into 3 pieces in the direction of diffusion, and then the magnetic properties of these magnets were tested. The magnets after diffusion were compared in terms of uniformity of properties, as shown in Table 4 below.

**Table 4 Comparison of uniformity of properties of magnets obtained in Example 2 and Comparative Example 2**

| Sample no. | Matrix before diffusion | Example 2 | Comparative Example 2 |
|---|---|---|---|
| | Hcj (kA/m, [kOe]) | Hcj (kA/m, [kOe]) | Hcj (kA/m, [kOe]) |
| 1# | 1233.80, [15.50] | 1535.48, [19.29] | 1503.64, [18.89] |
| 2# | 1233.80, [15.50] | 1472.60, [18.50] | 1397.78, [17.56] |
| 3# | 1234.60, [15.51] | 1537.08, [19.31] | 1498.07, [18.82] |

From Table 4, it can be seen that under the same weight gain conditions of heavy rare earth elements and diffusion process conditions, the difference in coercivity between a sample at an outermost layer position and a sample at a central position of the magnet obtained after diffusion in the diffusion direction in Example 2 is 63.68 kA/m [0.8 kOe], and the Hcj of the sample at a central position is 238.80 kA/m [3 kOe] higher than that of the matrix. The difference in coercivity between a sample at an outermost layer position and a sample at a central position of the magnet obtained after diffusion in the diffusion direction in Comparative Example 2 is 103.48 kA/m [1.3 kOe], and the Hcj of the sample at a central position is 163.98 kA/m [2.06 kOe] higher than that of the matrix. In addition, the property of the magnet at a central position after diffusion in Example 2 is 74.82 kA/m [0.94 kOe] higher than that of the magnet at a central position after diffusion in Comparative Example 2. From the above comparison it can be seen that the magnet in example 2 has a greater diffusion depth and is more uniformly diffused.

### Example 3

(S1) A total of 4 raw components, including a terbium hydride powder with an average particle size of 10 µm as a heavy rare earth diffusion source, a silicone rubber adhesive, ethylbenzene as solvent and a spherical boron nitride ceramic powder with an average particle size of 100 µm were used as raw materials of a heavy rare earth slurry. First, the terbium hydride powder was mixed with the spherical boron nitride powder, wherein the weight of the boron nitride ceramic powder was 10% of the weight of the terbium hydride powder. Then, the mixed powder was used as a diffusion source intermediate, and the diffusion source intermediate, the rubber adhesive and the benzene organic solvent were mixed in proportions of 80%, 6% and 14%, respectively, and stirred evenly to prepare the heavy rare earth slurry.

(S2) The heavy rare earth slurry was coated on two surfaces (10*10 mm) of a neodymium-iron-boron matrix with a size of 10*10*6 mm by spraying and dried to form a heavy rare earth coating with a special structure, wherein the weight ratio of heavy rare earth elements in the coating to the neodymium-iron-boron matrix was controlled to 1.0%. The neodymium-iron-boron matrix was obtained by performing processes such as melting, pulverizing, molding, sintering and aging to obtain an N55H brand blank and then performing machining and had a size of 10*10*6 mm.

(S3) The neodymium-iron-boron magnet coated with the heavy rare earth coating was subjected to diffusion and aging under the protection of an argon atmosphere, wherein the diffusion and aging processes were performed at a temperature of 950°C for 30 h and at a temperature of 600°C for 10 h, respectively. Then, overall magnetic properties of a product obtained after the diffusion was completed were tested.

The product obtained after the diffusion was completed was evenly cut into 5 pieces in a diffusion direction, and magnetic properties of magnets at different positions in the diffusion direction after the diffusion were tested. In order to fully illustrate technical advantages of the patent scheme compared with a traditional coating and diffusion scheme, Comparative Example 3 was also set below.

### Comparative Example 3

(S1) A total of 3 components, including a terbium hydride powder with an average particle size of 10 µm as a heavy rare earth diffusion source, a silicone rubber adhesive and ethylbenzene as solvent were used as raw materials of a heavy rare earth slurry. The terbium hydride powder, the rubber adhesive and the benzene organic solvent were mixed in proportions of 80%, 6% and 14%, respectively, and stirred evenly to prepare the heavy rare earth slurry.

(S2) The heavy rare earth slurry was coated on two surfaces (10*10 mm) of a neodymium-iron-boron matrix with a size of 10*10*6 mm by spraying and dried to form a heavy rare earth coating with a special structure, wherein the weight ratio of heavy rare earth elements in the coating to the neodymium-iron-boron matrix was controlled to 1.0%. The neodymium-iron-boron matrix was obtained by performing processes such as melting, pulverizing, molding, sintering and aging to obtain an N55H brand blank and then performing machining and had a size of 10*10*6 mm.

(S3) The neodymium-iron-boron magnet coated with the heavy rare earth coating was subjected to diffusion and aging under the protection of an argon atmosphere, wherein the diffusion and aging processes were performed at a temperature of 950°C for 30 h and at a temperature of 600°C for 10 h, respectively. Then, overall magnetic properties of a product obtained after the diffusion was completed were tested.

The product obtained after the diffusion was completed was evenly cut into 5 pieces in a diffusion direction, and magnetic properties of magnets at different positions in the diffusion direction after the diffusion were tested.

In order to compare the scratch resistance of heavy rare earth coatings in examples and comparative examples, a mutual friction experiment was carried out by enabling a sample coated with a heavy rare earth coating in Example 3 to get in contact with a coating surface of a sample coated with a heavy rare earth coating with a special structure in Comparative Example 3, proportions of exposed areas of matrices in total coating areas were calculated by statistics after heavy rare earth film layers on the surfaces of the samples in Example 3 and Comparative Example 3 were scratched, and statistical data were recorded in Table 5 and named as a scratch ratio.

In order to compare the shrinkage resistance of heavy rare earth coatings in examples and comparative examples in a high-temperature diffusion process, 100 pieces of diffusion samples in Example 3 and Comparative Example 3 were separately taken, proportions of samples having a shrinkage phenomenon of heavy rare earth film layers after diffusion in total statistical numbers were calculated by statistics, and statistical data were recorded in Table 5 and named as a shrinkage ratio.

Properties of a neodymium-iron-boron magnet before diffusion, overall properties of a neodymium-iron-boron magnet obtained after the diffusion was completed in Example 3 and overall properties of a neodymium-iron-boron magnet obtained after the diffusion was completed in Comparative Example 3 were compared, as shown in Table 5 below.

**Table 5 Comparison of properties of magnets obtained in Example 3 and Comparative Example 3**

| Sample | Scratch ratio | Shrinkage ratio | Br (T, [kGs]) | Hcj (kA/m, [kOe]) | Hk/Hcj |
|---|---|---|---|---|---|
| N55H magnet | / | / | 1.461, [14.61] | 1235.39, [15.52] | 0.989 |
| Example 3 | 0% | 0% | 1.438, [14.38] | 2133.28, [26.8] | 0.980 |
| Comparative Example 3 | 9% | 6% | 1.436, [14.36] | 2069.60, [26] | 0.975 |

From Table 5, it can be seen that the sample coated with a heavy rare earth coating having a special structure in Example 3 is not scratched in the mutual friction test with the sample coated with a heavy rare earth coating in Comparative Example 3, while the sample in Comparative Example 3 is scratched in a proportion of 9%, indicating that the heavy rare earth coating in Example 3 has a higher scratch resistance. In addition, the heavy rare earth coating on the surface of the sample in Comparative Example 3 exhibits a shrinkage phenomenon in a proportion of 6% in a high-temperature diffusion process, while the heavy rare earth coating on the surface of the sample in Example 3 does not exhibit a shrinkage phenomenon in a high-temperature diffusion process, indicating that the heavy rare earth coating with a special structure prepared in Example 3 has a higher shrinkage resistance than the heavy rare earth coating prepared in Comparative Example 3.

From Table 5, it can be seen that under the same heavy rare earth weight gain conditions, the content of Br in the magnet after diffusion in Example 3 is reduced by 0.023 T [0.23 kGs], the Hcj is improved by 897.89 kA/m [11.28 kOe], and the squareness is reduced by 0.009. The Br content in the magnet after diffusion in Comparative Example 3 is reduced by 0.025 T [0.25 kGs], the Hcj is improved by 834.21 kA/m [10.48 kOe] and the squareness is reduced by 0.014. From the above results it can be seen that the properties of neodymium-iron-boron magnets can be improved by the diffusion schemes in Example 3 and Comparative Example 3. However, under the same heavy rare earth weight gain conditions, the scheme in Example 3 has the advantage of improving the coercivity to a higher level.

The neodymium-iron-boron magnet before diffusion, the neodymium-iron-boron magnet obtained after diffusion in Example 3 and the neodymium-iron-boron magnet obtained after diffusion in Comparative Example 3 were each cut equally into 5 pieces in the direction of diffusion, and then the magnetic properties of these magnets were tested. The magnets after diffusion were compared in terms of uniformity of properties as shown in Table 6 below.

**Table 6 Comparison of uniformity of properties of magnets obtained in Example 3 and Comparative Example 3**

| Sample no. | Matrix before diffusion | Example 3 | Comparative Example 3 |
|---|---|---|---|
| | Hcj (kA/m, [kOe]) | Hcj (kA/m, [kOe]) | Hcj (kA/m, [kOe]) |
| 1# | 1234.60, [15.51] | 2165.12, [27.2] | 2137.26, [26.85] |
| 2# | 1233.80, [15.50] | 2077.56, [26.1] | 2005.92, [25.2] |
| 3# | 1234.60, [15.51] | 2029.80, [25.5] | 1934.28, [24.3] |
| 4# | 1233.80, [15.50] | 2085.52, [26.2] | 2029.80, [25.5] |
| 5# | 1234.60, [15.51] | 2165.12, [27.2] | 2133.28, [26.8] |

From Table 6, it can be seen that under same weight gain conditions of heavy rare earth elements and diffusion process conditions, the difference of the coercivity between a sample at an outermost layer position and a sample at a central position of the magnet obtained after diffusion in the diffusion direction in Example 3 is 135.32 kA/m [1.7 kOe], and the Hcj of the sample at a central position is 796 kA/m [10 kOe] higher than that of the matrix. The difference of the coercivity between a sample at an outermost layer position and a sample at a central position of the magnet obtained after diffusion in the diffusion direction in Comparative Example 3 is 202.98 kA/m [2.55 kOe], and the Hcj of the sample at a central position is 700.48 kA/m [8.8 kOe] higher than that of the matrix. In addition, the property of the magnet at a central position after diffusion in Example 3 is 95.52 kA/m [1.2 kOe] higher than that of the magnet at a central position after diffusion in Comparative Example 3. Through the above comparison, it can be seen that the magnet in Example 3 has a higher diffusion depth and is diffused more uniformly.

### Example 4

(S1) A total of 4 raw components, including a terbium hydride powder with an average particle size of 5 µm as a heavy rare earth diffusion source, a Polyvinyl chloride resin adhesive, s-butyl acetate as solvent and a spherical zirconia ceramic powder with an average particle size of 50 µm were used as raw materials of a heavy rare earth slurry. First, the terbium hydride powder was mixed with the spherical zirconia powder, wherein the weight of the zirconia ceramic powder was 30% of the weight of the terbium hydride powder. Then, the mixed powder was used as a diffusion source intermediate, and the diffusion source intermediate, the resin adhesive and the ester organic solvent were mixed in proportions of 60%, 8% and 32%, respectively, and stirred evenly to prepare the heavy rare earth slurry.

(S2) The heavy rare earth slurry was coated on two surfaces (10*10 mm) of a neodymium-iron-boron matrix with a size of 10*10*8 mm by spraying and dried to form a heavy rare earth coating with a special structure, wherein the weight ratio of heavy rare earth elements in the coating to the neodymium-iron-boron matrix was controlled to 1.5%. The neodymium-iron-boron matrix was obtained by performing processes such as melting, pulverizing, molding, sintering and aging to obtain an N42H brand blank and then performing machining and had a size of 10*10*8 mm.

(S3) The neodymium-iron-boron magnet coated with the heavy rare earth coating was subjected to diffusion and aging under vacuum conditions, wherein the diffusion and aging processes were performed at a temperature of 900°C for 40 h and at a temperature of 650°C for 8 h, respectively. Then, overall magnetic properties of a product obtained after the diffusion was completed were tested.

The product obtained after the diffusion was completed was evenly cut into 5 pieces in a diffusion direction, and magnetic properties of magnets at different positions in the diffusion direction after the diffusion were tested. In order to fully illustrate technical advantages of the patent scheme compared with a traditional coating and diffusion scheme, Comparative Example 4 was set below.

### Comparative Example 4

(S1) A total of 3 substances, including a terbium hydride powder with an average particle size of 5 µm as a heavy rare earth diffusion source, polyvinyl chloride resin adhesive and s-butyl acetate as solvent were used as raw materials of a heavy rare earth slurry. The terbium hydride powder, the resin adhesive and the ester organic solvent were mixed in proportions of 60%, 8% and 32%, respectively, and stirred evenly to prepare the heavy rare earth slurry.

(S2) The heavy rare earth slurry was coated on two surfaces (10*10 mm) of a neodymium-iron-boron matrix with a size of 10*10*8 mm by spraying and dried to form a heavy rare earth coating with a special structure, wherein the weight ratio of heavy rare earth elements in the coating to the neodymium-iron-boron matrix was controlled to 1.5%. The neodymium-iron-boron matrix was obtained by performing processes such as melting, pulverizing, molding, sintering and aging to obtain an N42H brand blank and then performing machining and had a size of 10*10*8 mm.

(S3) The neodymium-iron-boron magnet coated with the heavy rare earth coating was subjected to diffusion and aging under vacuum conditions, wherein the diffusion and aging processes were performed at a temperature of 900°C for 40 h and at a temperature of 650°C for 8 h, respectively. Then, overall magnetic properties of a product obtained after the diffusion was completed were tested.

The product obtained after the diffusion was completed was evenly cut into 5 pieces in a diffusion direction, and magnetic properties of magnets at different positions in the diffusion direction after the diffusion were tested.

In order to compare the scratch resistance of heavy rare earth coatings in examples and comparative examples, a mutual friction experiment was carried out by enabling a sample coated with a heavy rare earth coating in Example 4 to get in contact with a coating surface of a sample coated with a heavy rare earth coating with a special structure in Comparative Example 4, proportions of exposed areas of matrices in total coating areas were calculated by statistics after heavy rare earth film layers on the surfaces of the samples in Example 4 and Comparative Example 4 were scratched, and statistical data were recorded in Table 7 and named as a scratch ratio.

In order to compare the shrinkage resistance of heavy rare earth coatings in examples and comparative examples in a high-temperature diffusion process, 100 pieces of diffusion samples in Example 4 and Comparative Example 4 were separately taken, proportions of samples having a shrinkage phenomenon of heavy rare earth film layers after diffusion in total statistical numbers were calculated by statistics, and statistical data were recorded in Table 7 and named as a shrinkage ratio.

Properties of a neodymium-iron-boron magnet before diffusion, overall properties of a neodymium-iron-boron magnet obtained after the diffusion was completed in Example 4 and overall properties of a neodymium-iron-boron magnet obtained after the diffusion was completed in Comparative Example 4 were compared, as shown in Table 7 below.

**Table 7 Comparison of properties of magnets obtained in Example 4 and Comparative Example 4**

| Sample | Scratch ratio | Shrinkage ratio | Br (T, [kGs]) | Hcj (kA/m, [kOe]) | Hk/Hcj |
|---|---|---|---|---|---|
| uncoated magnet | / | / | 1.32, [13.20] | 1472.60, [18.05] | 0.981 |
| Example 4 | 0% | 0% | 1.292, [12.92] | 2388.00, [30] | 0.972 |
| Comparative Example 4 | 21% | 13% | 1.288, [12.88] | 2344.22, [29.45] | 0.968 |

From Table 7, it can be seen that the sample coated with a heavy rare earth coating having a special structure in Example 4 is not scratched in the mutual friction test with the sample coated with a heavy rare earth coating in Comparative Example 4, while the sample in Comparative Example 4 is scratched in a proportion of 21%, indicating that the heavy rare earth coating in Example 4 has a higher scratch resistance. In addition, the heavy rare earth coating on the surface of the sample in Comparative Example 4 has a shrinkage phenomenon in a proportion of 13% in a high temperature diffusion process, while the heavy rare earth coating on the surface of the sample in Example 4 has no shrinkage phenomenon in a high temperature diffusion process, indicating that the heavy rare earth coating with a special structure prepared in Example 4 has a higher shrinkage resistance than the heavy rare earth coating prepared in Comparative Example 4.

From Table 7, it can be seen that under the same heavy rare earth weight gain conditions, the content of Br in the magnet after diffusion in Example 4 is reduced by 0.028 T [0.28 kGs], the Hcj is improved by 951.22 kA/m [11.95 kOe], and the squareness is reduced by 0.009. The Br content in the magnet after diffusion in Comparative Example 4 is reduced by 0.032 T [0.32 kGs], the Hcj is improved by 907.44 kA/m [11.4 kOe] and the squareness is reduced by 0.013. From the above results it can be seen that the properties of neodymium-iron-boron magnets can be improved by the diffusion schemes in Example 4 and Comparative Example 4. However, under the same heavy rare earth weight gain conditions, the scheme in Example 4 has the advantage of improving the coercivity to a higher level.

The neodymium-iron-boron magnet before diffusion, the neodymium-iron-boron magnet obtained after diffusion in Example 4 and the neodymium-iron-boron magnet obtained after diffusion in Comparative Example 4 were each cut equally into 5 pieces in the direction of diffusion, and then the magnetic properties of these magnets were tested. The magnets after diffusion were compared in terms of uniformity of properties as shown in Table 8 below.

**Table 8 Comparison of uniformity of properties of magnets obtained in Example 4 and Comparative Example 4**

| Sample number | Matrix before diffusion | Example 1 | Comparative Example 1 |
|---|---|---|---|
| | Hcj (kA/m, [kOe]) | Hcj (kA/m, [kOe]) | Hcj (kA/m, [kOe]) |
| 1# | 1433.60, [18.01] | 2469.19, [31.02] | 2451.68, [30.8] |
| 2# | 1432.80, [18.00] | 2317.95, [29.12] | 2268.60, [28.5] |
| 3# | 1433.60, [18.01] | 2245.52, [28.21] | 2157.16, [27.1] |
| 4# | 1434.40, [18.02] | 2309.99, [29.02] | 2276.56, [28.6] |
| 5# | 1432.80, [18.00] | 2468.40, [31.01] | 2459.64, [30.9] |

From Table 8, it can be seen that under the same heavy rare earth weight gain conditions and diffusion process conditions, the difference in coercivity between a sample at an outermost layer position and a sample at a central position of the magnet obtained after diffusion in the diffusion direction in Example 4 is 223.68 [2.81 kOe], and the Hcj of the sample at a central position is 797.59 kA/m [10.02 kOe] higher than that of the matrix. The difference in coercivity between a sample at an outermost layer position and a sample at a central position of the magnet obtained after diffusion in the diffusion direction in Comparative Example 4 is 298.50 kA/m [3.75 kOe], and the Hcj of the sample at a central position is 723.56 kA/m [9.09 kOe] higher than that of the matrix. In addition, the property of the magnet at a central position after diffusion in Example 4 is 88.36 kA/m [1.11 kOe] higher than that of the magnet at a central position after diffusion in Comparative Example 4. From the above comparison it can be seen that the magnet in example 4 has a greater diffusion depth and is more uniformly diffused.

## Claims

1. A method for improving the coercivity of a neodymium-iron-boron magnet, comprising the following steps:
(S1) subjecting a heavy rare earth diffusion source powder, an organic adhesive, a spherical high-temperature resistant ceramic powder and an organic solvent to mixing and stirring to prepare a heavy rare earth slurry, wherein the particle size of the spherical high-temperature resistant ceramic powder is 5 to 10 times of that of the diffusion source powder, and the weight of the spherical high-temperature resistant ceramic powder is 10% to 30% of that of the heavy rare earth diffusion source powder;
(S2) coating a surface of a neodymium-iron-boron magnet with the heavy rare earth slurry and drying the heavy rare earth slurry to form a heavy rare earth coating; and
(S3) subjecting the neodymium-iron-boron magnet coated with the heavy rare earth coating to high-temperature diffusion and aging treatment under vacuum or argon protection conditions.

2. The method for improving the coercivity of a neodymium-iron-boron magnet according to claim 1, wherein in step (S1), the heavy rare earth diffusion source powder is at least one of a pure terbium powder, a pure dysprosium powder, a dysprosium hydride powder and a terbium hydride powder, and the heavy rare earth diffusion source powder has an average particle size in a range of 2 to 10 µm measured by laser diffraction.

3. The method for improving the coercivity of a neodymium-iron-boron magnet according to claim 1 or 2, wherein in step (S1), the organic adhesive is a resin adhesive or a rubber adhesive.

4. The method for improving the coercivity of a neodymium-iron-boron magnet according to any one of the preceding claims, wherein in step (S1), the organic solvent is acetone, s-butyl acetate, ethylbenzene or a combination thereof.

5. The method for improving the coercivity of a neodymium-iron-boron magnet according to any one of the preceding claims, wherein in step (S1), the spherical high-temperature resistant ceramic powder is at least one of a spherical alumina ceramic powder, a spherical zirconia ceramic powder and a spherical boron nitride ceramic powder.

6. The method for improving the coercivity of a neodymium-iron-boron magnet according to any one of the preceding claims, wherein the spherical high-temperature resistant ceramic powder has an average particle size in a range of 10 to 100 µm measured by laser diffraction.

7. The method for improving the coercivity of a neodymium-iron-boron magnet according to any one of the preceding claims, wherein in step (S1), the total weight of the heavy rare earth diffusion source powder and the spherical high-temperature resistant ceramic powder is 40% to 80% of the weight of the heavy rare earth slurry, the weight of the organic adhesive is 5% to 10% of the weight of the heavy rare earth slurry, and the organic solvent is the residual.

8. The method for improving the coercivity of a neodymium-iron-boron magnet according to any one of the preceding claims, wherein in step (S2), the heavy rare earth slurry is coated by screen printing or spraying.

9. The method for improving the coercivity of a neodymium-iron-boron magnet according to any one of the preceding claims, wherein in step (S2), the weight of the heavy rare earth diffusion source powder in the heavy rare earth coating coated on the surface of the neodymium-iron-boron magnet is 0.3% to 1.5% of the weight of the neodymium-iron-boron magnet.

10. The method for improving the coercivity of a neodymium-iron-boron magnet according to any one of the preceding claims, wherein in step (S3), the high-temperature diffusion is performed at a temperature of 850 to 950 °C for 3 to 48 h.

11. The method for improving the coercivity of a neodymium-iron-boron magnet according to any one of the preceding claims, wherein in step (S3), the aging treatment is performed at a temperature of 450 to 650°C for 3 to 10 h.

## Patentansprüche

1. Verfahren zur Verbesserung der Koerzitivkraft eines Neodym-Eisen-Bor-Magneten, umfassend die folgenden Schritte:
(S1) Unterwerfen eines schweren Seltenerd-Diffusionsquellenpulvers, eines organischen Klebstoffs, eines kugelförmigen hochtemperaturbeständigen Keramikpulvers und eines organischen Lösungsmittels einem Misch- und Rührvorgang, um eine schwere Seltenerd-Aufschlämmung vorzubereiten, wobei die Partikelgröße des kugelförmigen hochtemperaturbeständigen Keramikpulvers das 5- bis 10-fache derjenigen des Diffusionsquellenpulvers beträgt und das Gewicht des kugelförmigen hochtemperaturbeständigen Keramikpulvers 10% bis 30% desjenigen des schweren Seltenerd-Diffusionsquellenpulvers beträgt;
(S2) Beschichten einer Oberfläche eines Neodym-Eisen-Bor-Magneten mit der schweren Seltenerd-Aufschlämmung und Trocknen der schweren Seltenerd-Aufschlämmung, um eine schwere Seltenerd-Beschichtung zu bilden; und
(S3) Unterwerfen des mit der schweren Seltenerd-Beschichtung beschichteten Neodym-Eisen-Bor-Magneten einer Hochtemperatur-Diffusions- und Alterungsbehandlung unter Vakuum- oder Argonschutzbedingungen.

2. Verfahren zur Verbesserung der Koerzitivkraft eines Neodym-Eisen-Bor-Magneten nach Anspruch 1, wobei in Schritt (S1) das schwere Seltenerd-Diffusionsquellenpulver mindestens eines von einem reinen Terbiumpulver, einem reinen Dysprosiumpulver, einem Dysprosiumhydridpulver und einem Terbiumhydridpulver ist und das schwere Seltenerd-Diffusionsquellenpulver eine durchschnittliche Partikelgröße im Bereich von 2 µm bis 10 µm, gemessen durch Laserbeugung, aufweist.

3. Verfahren zur Verbesserung der Koerzitivkraft eines Neodym-Eisen-Bor-Magneten nach Anspruch 1 oder 2, wobei in Schritt (S1) der organische Klebstoff ein Harzklebstoff oder ein Kautschukklebstoff ist.

4. Verfahren zur Verbesserung der Koerzitivkraft eines Neodym-Eisen-Bor-Magneten nach einem der vorstehenden Ansprüche, wobei in Schritt (S1) das organische Lösungsmittel Aceton, s-Butylacetat, Ethylbenzol oder eine Kombination davon ist.

5. Verfahren zur Verbesserung der Koerzitivkraft eines Neodym-Eisen-Bor-Magneten nach einem der vorstehenden Ansprüche, wobei in Schritt (S1) das kugelförmige hochtemperaturbeständige Keramikpulver mindestens eines von einem kugelförmigen Aluminiumoxid-Keramikpulver, einem kugelförmigen Zirkonoxid-Keramikpulver und einem kugelförmigen Bornitrid-Keramikpulver ist.

6. Verfahren zur Verbesserung der Koerzitivkraft eines Neodym-Eisen-Bor-Magneten nach einem der vorstehenden Ansprüche, wobei das kugelförmige hochtemperaturbeständige Keramikpulver eine durchschnittliche Partikelgröße im Bereich von 10 µm bis 100 µm, gemessen durch Laserbeugung, aufweist.

7. Verfahren zur Verbesserung der Koerzitivkraft eines Neodym-Eisen-Bor-Magneten nach einem der vorstehenden Ansprüche, wobei in Schritt (S1) das Gesamtgewicht des schweren Seltenerd-Diffusionsquellenpulvers und des kugelförmigen hochtemperaturbeständigen Keramikpulvers 40% bis 80% des Gewichts der schweren Seltenerd-Aufschlämmung beträgt, das Gewicht des organischen Klebstoffs 5% bis 10% des Gewichts der schweren Seltenerd-Aufschlämmung beträgt und das organische Lösungsmittel den Rest ausmacht.

8. Verfahren zur Verbesserung der Koerzitivkraft eines Neodym-Eisen-Bor-Magneten nach einem der vorstehenden Ansprüche, wobei in Schritt (S2) die schwere Seltenerd-Aufschlämmung durch Siebdruck oder Sprühen beschichtet wird.

9. Verfahren zur Verbesserung der Koerzitivkraft eines Neodym-Eisen-Bor-Magneten nach einem der vorstehenden Ansprüche, wobei in Schritt (S2) das Gewicht des schweren Seltenerd-Diffusionsquellenpulvers in der schweren Seltenerd-Beschichtung, die auf die Oberfläche des Neodym-Eisen-Bor-Magneten aufgetragen ist, 0,3% bis 1,5% des Gewichts des Neodym-Eisen-Bor-Magneten beträgt.

10. Verfahren zur Verbesserung der Koerzitivkraft eines Neodym-Eisen-Bor-Magneten nach einem der vorstehenden Ansprüche, wobei in Schritt (S3) die Hochtemperaturdiffusion bei einer Temperatur von 850°C bis 950°C für 3 bis 48 Stunden durchgeführt wird.

11. Verfahren zur Verbesserung der Koerzitivkraft eines Neodym-Eisen-Bor-Magneten nach einem der vorstehenden Ansprüche, wobei in Schritt (S3) die Alterungsbehandlung bei einer Temperatur von 450°C bis 650°C für 3 bis 10 Stunden durchgeführt wird.

## Revendications

1. Procédé d'amélioration de la coercivité d'un aimant néodyme-fer-bore, comprenant les étapes suivantes :
(S1) soumettre une poudre de source de diffusion de terres rares lourdes, un adhésif organique, une poudre de céramique sphérique résistante à haute température et un solvant organique à un mélange et à une agitation pour préparer une pâte de terres rares lourdes, dans laquelle la taille des particules de la poudre de céramique sphérique résistante à haute température est de 5 à 10 fois celle de la poudre de source de diffusion et le poids de la poudre de céramique sphérique résistante à haute température est de 10 % à 30 % de celui de la poudre de source de diffusion de terres rares lourdes ;
(S2) revêtir une surface d'un aimant néodyme-fer-bore de la pâte de terres rares lourdes et sécher la pâte de terres rares lourdes pour former un revêtement en terres rares lourdes ; et
(S3) soumettre l'aimant néodyme-fer-bore revêtu du revêtement en terres rares lourdes à un traitement de diffusion et de vieillissement à haute température sous conditions de protection sous vide ou sous argon.

2. Procédé d'amélioration de la coercivité d'un aimant néodyme-fer-bore selon la revendication 1, dans lequel, à l'étape (S1), la poudre de source de diffusion de terres rares lourdes est au moins l'une parmi une poudre de terbium pur, une poudre de dysprosium pur, une poudre d'hydrure de dysprosium et une poudre d'hydrure de terbium, et la poudre de source de diffusion de terres rares lourdes présente une taille moyenne des particules comprise dans une plage de 2 à 10 µm mesurée par diffraction laser.

3. Procédé d'amélioration de la coercivité d'un aimant néodyme-fer-bore selon la revendication 1 ou 2, dans lequel, à l'étape (S1), l'adhésif organique est un adhésif à la résine ou un adhésif au caoutchouc.

4. Procédé d'amélioration de la coercivité d'un aimant néodyme-fer-bore selon l'une quelconque des revendications précédentes, dans lequel, à l'étape (S1), le solvant organique est l'acétone, l'acétate de s-butyle, l'éthylbenzène ou une combinaison de ceux-ci.

5. Procédé d'amélioration de la coercivité d'un aimant néodyme-fer-bore selon l'une quelconque des revendications précédentes, dans lequel, à l'étape (S1), la poudre de céramique sphérique résistante à haute température est au moins l'une parmi une poudre de céramique d'alumine sphérique, une poudre de céramique de zircone sphérique et une poudre de céramique de nitrure de bore sphérique.

6. Procédé d'amélioration de la coercivité d'un aimant néodyme-fer-bore selon l'une quelconque des revendications précédentes, dans lequel la poudre de céramique sphérique résistante à haute température présente une taille moyenne des particules comprise dans une plage de 10 à 100 µm mesurée par diffraction laser.

7. Procédé d'amélioration de la coercivité d'un aimant néodyme-fer-bore selon l'une quelconque des revendications précédentes, dans lequel, à l'étape (S1), le poids total de la poudre de source de diffusion de terres rares lourdes et de la poudre de céramique sphérique résistante à haute température est de 40 % à 80 % du poids de la pâte de terres rares lourdes, le poids de l'adhésif organique est de 5 % à 10 % du poids de la pâte de terres rares lourdes et le solvant organique constitue le reste.

8. Procédé d'amélioration de la coercivité d'un aimant néodyme-fer-bore selon l'une quelconque des revendications précédentes, dans lequel, à l'étape (S2), la pâte de terres rares lourdes est revêtue par sérigraphie ou pulvérisation.

9. Procédé d'amélioration de la coercivité d'un aimant néodyme-fer-bore selon l'une quelconque des revendications précédentes, dans lequel, à l'étape (S2), le poids de la poudre de source de diffusion de terres rares lourdes dans le revêtement en terres rares lourdes revêtu sur la surface de l'aimant néodyme-fer-bore est de 0,3 % à 1,5 % du poids de l'aimant néodyme-fer-bore.

10. Procédé d'amélioration de la coercivité d'un aimant néodyme-fer-bore selon l'une quelconque des revendications précédentes, dans lequel, à l'étape (S3), le traitement de diffusion à haute température est effectué à une température de 850 à 950 °C pendant 3 à 48 heures.

11. Procédé d'amélioration de la coercivité d'un aimant néodyme-fer-bore selon l'une quelconque des revendications précédentes, dans laquelle, à l'étape (S3), le traitement de vieillissement est effectué à une température de 450 à 650 °C pendant 3 à 10 heures.
